

1

3,464,817

ALLOY COMPOSITION AND METHOD OF FORMING THE SAME

Emil S. Griffiths, Albany, N.Y., assignor to CMP Industries, Inc., Albany, N.Y., a corporation of New York  
No Drawing. Filed Mar. 17, 1966, Ser. No. 535,027  
Int. Cl. C22c 19/00

U.S. Cl. 75—171

15 Claims

ABSTRACT OF THE DISCLOSURE

An alloy suitable for use in forming dentures and other dental prostheses contains, in weight percent, about 10% to 28% chromium, about 5% to 12% molybdenum, about 3% to 7% manganese, about 0.2% to 2% beryllium, about 2% to 6% aluminum, up to about 22% cobalt and the balance essentially nickel. This alloy is characterized by high strength, toughness, good ductility, good fluidity in the molten state, and controlled shrinkage when cast. These properties cause the alloy to abrade readily for ease of polishing, permit deformation by bending without fracture when necessary to mechanically adjust parts formed of the alloy in dental prostheses, and allow the casting of thin or attenuated sections and other pieces within close tolerances. The alloy preferably is formed by melting the alloying elements in a preferred sequence and maintaining selected alloying elements beneath the surface of the molten pool to prevent oxidation.

My invention relates to alloy compositions and the method of forming the same and particularly to alloy compositions suitable for the production of dental prostheses. Also the invention relates to the method for the production of such alloy compositions.

Dental alloy compositions adapted for prosthetic articles are discussed in United States Patent No. 2,631,095, granted Mar. 10, 1953, for "Alloy Adapted for Prosthetic Articles." The alloy system discussed in U.S. Patent No. 2,631,095 employs chromium, molybdenum, beryllium, manganese and copper with the balance of the alloy being a combination of cobalt and nickel. However, in the past, as in the alloy described in U.S. Patent No. 2,631,095, ease of polishing, although a desirable property, had to be sacrificed in order to provide an alloy with sufficient yield strength.

Because the prosthetic articles or appliances cast from the alloy are used in the mouth, the space available for their insertion is always limited and for this reason the alloy must be exceptionally strong. When casting partial denture prostheses, high yield strength is essential if the alloy is to function properly since the clasps used to retain the appliance are small in cross section and the retention provided for mounting the artificial teeth is also thin and attenuated. Ordinarily, as yield strength values are increased, hardness also increases but ease of polishing decreases.

Yield strength and ease of polishing are not the only important characteristics. Ductility is important since the clasps must permit adjustment without the risk of shearing or breaking. In order to achieve an accurate fit when the appliance is inserted in the mouth, the net casting shrinkage must be controlled within rather limited tolerances. Further, because the appliances are constructed with rather thin attenuated areas of relatively small cross section, the alloy must be highly fluid at casting temperature so that it will flow readily into these restricted openings and not form voids or cavities therein which would render the appliance unusable. This is true especially with

2

full denture prostheses or veneer castings for full bridge work.

It is an object of my invention to overcome the difficulties heretofore encountered and it is a primary object of my invention to provide an alloy composition suitable for use as a dental prosthesis which is readily abraded and polished but which will maintain hardness, yield strength, and sufficient ductility, without the risk of shearing or breaking the appliance when it is adjusted for insertion in the mouth.

It is also an object of my invention to provide an alloy which will maintain a high luster after it is completed and which will resist discoloration after prolonged use.

My invention generally contemplates providing an alloy composition suitable for the production of dental prostheses in which a plurality of elements in desired proportions comprise chromium, molybdenum, manganese, beryllium, aluminum, cobalt and nickel. The alloy is characterized in that it is easily cast into an appliance which has increased yield strength and improved ductility, but still possesses the ability to abrade readily for ease of polishing. Further, the novel combination of the elements comprising the alloy produces an alloy in which substantially all of the elements are combined with a minimum loss of the alloy due to oxide formation.

I have found in my new alloy composition that unexpected results are obtained by alteration of the alloy system disclosed in U.S. Patent No. 2,631,095, referred to above, so as to achieve the desired characteristics disclosed therein and with the added improvement in the ability of the new alloy to abrade readily so as to permit ease of polishing of the prosthetic articles without the risk of shearing or breaking the appliance when it is adjusted for insertion in the mouth. By changing the alloy system and utilizing aluminum in place of copper, and reducing the cobalt content with disregard of the cobalt-nickel ratio as taught in U.S. Patent No. 2,631,095, unexpected results are achieved. Thus by employing an aluminum content not in excess of 6% and a cobalt content not in excess of 22% and without the necessity of maintaining a nickel-cobalt ratio, an improved alloy system useful for full and partial prosthetic articles is achieved. As stated previously, my new alloy is readily abraded and polished without any loss of the necessary physical characteristics that must be present for prosthetic articles of this type.

The elements comprising my new alloy composition are set forth below and their percentages, by weight, of the total composition are:

|            | Percent |
|------------|---------|
| Chromium   | 10-28   |
| Molybdenum | 0-12    |
| Manganese  | 0-7     |
| Beryllium  | 0.2-2   |
| Aluminum   | 0-6     |
| Cobalt     | 0-22    |
| Nickel     | Balance |

The preferred ranges of elements forming my improved alloy composition are set forth below and their percentages, by weight, of the total composition are:

|            | Percent                        |
|------------|--------------------------------|
| Chromium   | 12-24                          |
| Molybdenum | 5-7                            |
| Manganese  | 3-5                            |
| Beryllium  | 0.5-1                          |
| Aluminum   | 2-4                            |
| Cobalt     | 0-3 and 12-15 or 3-6 and 18-22 |
| Nickel     | Balance                        |

It is to be noted that the cobalt in the preferred composition lies within the ranges of from approximately 0 to 3% and 12 to 15%. It has been found that such an

alloy composition having the percentage of cobalt set forth therein exhibits excellent qualities and physical characteristics for partial dentures while the ranges of cobalt of approximately 3 to 6% and 18 to 22% exhibit excellent qualities and physical characteristics for full dentures.

An alloy suitable for use as a partial denture is characterized by its ability to adjust without shearing; that is, the attenuations which are the clasping or clamping means for holding the denture in the mouth must be sufficiently ductile and resilient so that when the dental appliance is adjusted for use these attenuations will not shear. When a full denture is employed it is not necessary for it to exhibit the degree of ductility and resiliency that is required in a partial denture. However, the alloy employed, whether used as a partial or full dental appliance, must have a characteristic of being capable of exhibiting sufficient casting fluidity, i.e., the ability to form thin, resilient and ductile films when employed as a full denture and the ability to flow readily into cavities forming the attenuations or clasping means in a partial denture. All of these characteristics are exhibited by my new alloy.

In making my alloy composition it is preferred that the elements be combined by employing induction or high frequency heating, although other accepted heating procedures may be employed.

I have found that in forming my alloy certain of the elements when added to the melt in a preferred sequence, produce an alloy having the desired physical characteristics which include high yield strength, increased ductility, sufficient hardness, and the ability to abrade readily for ease of polishing. When charging a crucible with my improved composition, the nickel is added first and a partially molten pool is formed. When the nickel is sufficiently liquid to permit forcing additional material below the surface of the molten pool, molybdenum is added and immediately forced beneath the surface so that it will not be exposed to the air and be lost by oxide formation. It should be noted that the molybdenum does not melt but rather dissolves in the liquid pool. However, it would volatilize as an oxide if heated in air. Thus, it is essential that the molybdenum be completely immersed if good recovery of the molybdenum is to be obtained.

The temperature of the molten pool of nickel will generally be 2650° F. before the addition of molybdenum as described above. However, where prealloyed materials are used as part of the alloy mix the temperature of the melt prior to the addition of molybdenum can be as low as 2400° F.

The chromium is added next. This, too, is forced under the surface of the liquid pool as much as possible. Since the bulk of the chromium added is much greater than that of the molybdenum, it may cause the nickel which has already liquified to freeze. No further additions are made until the pool again starts to liquify.

When this occurs the aluminum is added. The aluminum is low melting. However, it has been found that when it is added to a melt having a relatively high nickel content, a high melting nickel aluminum compound is formed and unless sufficient time is allowed for the high melting components to dissolve and disperse throughout the melt, serious segregation of the high melting compound may occur. The reaction causing the formation of the high melting compound is apparently exothermic and the liberation of this heat helps to further liquefy the pool and stimulate the solution of both the chromium and the aluminum.

In alloys which are to contain cobalt, the cobalt is added at this time.

After the melt has been heated for a sufficient time to completely dissolve all of the components and form a homogeneous pool, the sides of the crucible are scraped down to remove any dross which floats to the surface and can be skimmed off. At this time the melt is at a tempera-

ture of approximately 2700° F. and is deoxidized with an addition of calcium-silicon-manganese. The reaction products for this deoxidation are skimmed from the surface in order to leave the surface clean.

5 The manganese is then added. This dissolves very quickly. Any slight dross which forms is skimmed from the surface so that the pool again is clean.

The beryllium addition is then made. Because of the low specific gravity of the beryllium it will tend to float on the surface and the operator must use a skimming rod to force it beneath the surface of the molten pool.

10 The temperature of the melt is checked and heating continued until a temperature of 2800° F. is reached. At this point the sides of the crucible are again scraped to remove any dross and the surface of the pool skimmed to remove the material which floats to the surface. The alloy can then be poured.

15 The following examples illustrate alloy compositions and their percentages, by weight, of the total composition when made in accordance with the method set forth above:

#### EXAMPLE 1

|             | Percent |
|-------------|---------|
| 25 Chromium | 15      |
| Molybdenum  | 5       |
| Manganese   | 3.5     |
| Beryllium   | 0.8     |
| Aluminum    | 3.0     |
| 30 Cobalt   | 0       |
| Nickel      | Balance |

#### EXAMPLE 2

|             | Percent |
|-------------|---------|
| 35 Chromium | 15      |
| Molybdenum  | 10      |
| Manganese   | 3.5     |
| Beryllium   | 0.8     |
| Aluminum    | 3.0     |
| 40 Cobalt   | 0       |
| Nickel      | Balance |

#### EXAMPLE 3

|             | Percent |
|-------------|---------|
| 45 Chromium | 15.0    |
| Molybdenum  | 5.0     |
| Manganese   | 3.5     |
| Beryllium   | 0.8     |
| Aluminum    | 3.0     |
| 50 Cobalt   | 10.0    |
| Nickel      | Balance |

55 As previously indicated, and set forth in Examples 1-3, alloy compositions made in accordance with the method described above are suitable for use as partial dentures and exhibit the improved physical characteristics as set forth hereinabove.

#### EXAMPLE 4

|             | Percent |
|-------------|---------|
| 60 Chromium | 10.0    |
| Molybdenum  | 5.0     |
| Manganese   | 3.5     |
| Beryllium   | 0.8     |
| Aluminum    | 3.0     |
| 65 Cobalt   | 0       |
| Nickel      | Balance |

#### EXAMPLE 5

|             | Percent |
|-------------|---------|
| 70 Chromium | 15.0    |
| Molybdenum  | 0       |
| Manganese   | 3.5     |
| Beryllium   | 0.8     |
| Aluminum    | 3.0     |
| Cobalt      | 0       |
| 75 Nickel   | Balance |

**5**  
**EXAMPLE 6**

|            | Percent |
|------------|---------|
| Chromium   | 15.0    |
| Molybdenum | 5.0     |
| Manganese  | 3.5     |
| Beryllium  | 0.8     |
| Aluminum   | 0       |
| Cobalt     | 0       |
| Nickel     | Balance |

**EXAMPLE 7**

|            | Percent |
|------------|---------|
| Chromium   | 15.0    |
| Molybdenum | 5.0     |
| Manganese  | 3.5     |
| Beryllium  | 0.8     |
| Aluminum   | 3.0     |
| Cobalt     | 20.0    |
| Nickel     | Balance |

As previously indicated and as set forth in the alloy compositions of Examples 4-7, alloy compositions made in accordance with the method described above are suitable for use as full dentures and exhibit the improved physical characteristics as set forth hereinabove.

be helpful in understanding my invention. Tables I and II show variations in physical characteristics achieved by varying the content of the ingredients of the alloy composition when made in accordance with the method described herein. The variations are illustrated relative to the physical characteristics of Rockwell hardness, resilience, ductility (toughness), liquidus (lowest temperature in degrees F. at which the alloy composition is completely liquid), and the preferred use of the particular alloy composition with regard to its usefulness as a partial or full denture, or both. Also in Table II the alloys have been grouped on the basis of the ingredient being varied so that the effect of the variation on Rockwell hardness, resilience, toughness, and in some instances the liquidus temperature is readily apparent. As is apparent from the table, these properties do not vary linearly with changes in the amount of the ingredients employed.

TABLE I.—COMPOSITION

| Alloy No. | Ni   | Co | Cr   | Mo   | Mn  | Be  | Al  |
|-----------|------|----|------|------|-----|-----|-----|
| 60        | 65.7 | 0  | 22.0 | 5.0  | 3.5 | 0.8 | 3.0 |
| 76        | 60.0 | 0  | 27.7 | 5.0  | 3.5 | 0.8 | 3.0 |
| 79        | 62.7 | 0  | 15.0 | 15.0 | 3.5 | 0.8 | 3.0 |
| 82        | 73.5 | 0  | 15.0 | 5.0  | 3.5 | 0   | 3.0 |
| 90        | 71.9 | 0  | 15.0 | 5.0  | 3.5 | 1.6 | 3.0 |
| 92        | 82.7 | 0  | 5.0  | 5.0  | 3.5 | 0.8 | 3.0 |
| 95        | 76.2 | 0  | 15.0 | 5.0  | 0   | 0.8 | 3.0 |
| 96        | 69.2 | 0  | 15.0 | 5.0  | 7.0 | 0.8 | 3.0 |
| 101       | 71.5 | 0  | 15.0 | 5.0  | 3.5 | 2.0 | 3.0 |
| 103       | 69.7 | 0  | 15.0 | 5.0  | 3.5 | 0.8 | 6.0 |

TABLE II

| Alloy No. varied, percent | Rockwell hardness | Resilience     | Toughness      | Degrees F. liquidus | Use               |
|---------------------------|-------------------|----------------|----------------|---------------------|-------------------|
| Chromium                  |                   |                |                |                     |                   |
| Ex. 1..... 15             | C32               | Excellent..... | Excellent..... |                     | Partial.          |
| 92..... 5                 | C28               | Soft.....      | do.....        | 2,730               | Full.             |
| Ex. 4..... 10             | 28                | do.....        | do.....        | 2,550               | Do.               |
| 60..... 22                | 27                | Good.....      | Fair-poor..... | 2,530               | Do.               |
| 76..... 27.7              | 29                | Fair.....      | Good.....      |                     | Do.               |
| Molybdenum                |                   |                |                |                     |                   |
| Ex. 5..... 0              | C24               | Dead.....      | Excellent..... |                     | Do.               |
| Ex. 2..... 10             | 33                | Very good..... | Very good..... |                     | Partial.          |
| 79..... 15                | 44                | Excellent..... | None.....      |                     | Full.             |
| Beryllium                 |                   |                |                |                     |                   |
| 82..... 0                 | B90               | Dead.....      | Excellent..... |                     | Do.               |
| 90..... 1.6               | C35               | Very Good..... | Good.....      | 2,460               | Partial.          |
| 101..... 2.0              | 34                | do.....        | Fair-good..... |                     | Do.               |
| Aluminum                  |                   |                |                |                     |                   |
| Ex. 6..... 0              | B89               | Very dead..... | Excellent..... | 2,670               | Full.             |
| 103..... 6.0              | C41               | Excellent..... | None.....      |                     | Do.               |
| Manganese                 |                   |                |                |                     |                   |
| 95..... 0                 | C30               | Fair-soft..... | Excellent..... | 2,575               | Do.               |
| 96..... 7.0               | 28                | Good.....      | Fair.....      | 2,485               | Partial.          |
| Cobalt                    |                   |                |                |                     |                   |
| Ex. 8..... 5.0            | C28               | Fair-soft..... | Excellent..... | 2,550               | Full and partial. |
| Ex. 3..... 10             | 30                | Excellent..... | do.....        | 2,535               | Partial.          |
| Ex. 7..... 20             | 14                | Dead.....      | do.....        |                     | Full.             |

**EXAMPLE 8**

|            | Percent |
|------------|---------|
| Chromium   | 15.0    |
| Molybdenum | 5.0     |
| Manganese  | 3.5     |
| Beryllium  | 0.8     |
| Aluminum   | 3.0     |
| Cobalt     | 5.0     |
| Nickel     | Balance |

The composition of Example 8 is an example of an alloy which is suitable for use both as a partial or full denture and exhibits the improved characteristics of my new alloy composition.

The alloy compositions set forth in Table I below and when made in accordance with the method described herein and when cast into a dental appliance exhibit the improved and unexpected physical characteristics concerning my new alloy composition when the dental appliance is used for its preferred use.

A consideration of the alloy compositions set forth in the foregoing examples and in Tables I and II below will

55 I claim:

1. A method of forming an alloy suitable for casting dental prostheses having high strength and the ability to abrade readily for ease of polishing and sufficient ductile characteristics for readily adjusting said prostheses comprising melting said alloy by heating, sequentially controlling the addition of the elements forming said alloy which consists essentially of about 10% to 28% chromium, about 5% to 12% molybdenum, about 3% to 7% manganese, about 0.2% to 2% beryllium, about 2% to 6% aluminum, up to about 22% cobalt and the balance essentially nickel, said addition being accomplished by charging nickel into a crucible; heating the crucible to melt the nickel and form a molten pool thereof; adding the molybdenum so that it is submerged in the molten nickel pool; sequentially adding chromium, aluminum, cobalt and manganese to the nickel and molybdenum molten pool and then adding the beryllium so that it is maintained beneath the surface of the formed molten pool so as to prevent oxide formation and loss of beryllium in the final

alloy mixture whereby a substantially homogeneous mixture of molten elements are formed.

2. The method of forming an alloy as set forth in claim 1 wherein said alloy mixture is melted by induction heating and then cast into a desired dental prosthesis.

3. An alloy suitable for use in forming dental prostheses and the like and consisting essentially, in weight percent, of about 10% to 28% chromium, about 5% to 12% molybdenum, about 3% to 7% manganese, about 0.2% to 2% beryllium, about 2% to 6% aluminum, up to about 22% cobalt and the balance essentially nickel; said alloy being characterized by high strength and good toughness and ductility, good fluidity in the molten state, and controlled shrinkage when cast, whereby the alloy will abrade readily for ease of polishing, can be substantially deformed by bending without fracture when necessary to mechanically adjust parts formed of the alloy in dentures or other prostheses, and is capable of forming thin or attenuated sections within close tolerances when cast.

4. An alloy suitable in forming partial dentures in accordance with claim 3 which consists essentially of about 15% chromium, about 10% molybdenum, about 3.5% manganese, about 0.8% beryllium, about 3.0% aluminum, and the balance essentially nickel.

5. An alloy suitable in forming partial dentures in accordance with claim 3 which contains up to about 3% cobalt.

6. An alloy suitable in forming partial dentures in accordance with claim 3 which contains about 12% to 15% cobalt.

7. An alloy suitable in forming full dentures in accordance with claim 3 which contains about 3% to 6% cobalt.

8. An alloy suitable in forming full dentures in accordance with claim 3 which contains about 18% to 22% cobalt.

9. An alloy particularly suitable for use in making dental prostheses and the like and consisting essentially, in weight percent, of about 12% to 24% chromium, about 5% to 7% molybdenum, about 3% to 5% manganese, about 0.5% to 1% beryllium, about 2% and 4% aluminum, up to about 22% cobalt and the balance essentially nickel; said alloy being characterized by high strength and good toughness and ductility, good fluidity in the molten state and controlled shrinkage when cast, whereby the alloy will abrade readily for ease of polishing

can be substantially deformed by bending without fracture when necessary to mechanically adjust parts formed of the alloy in dentures or other dental prostheses, and is capable of forming thin or attenuated sections within close tolerances when cast.

5 10. An alloy suitable in forming partial dentures in accordance with claim 9 which consists essentially of about 15% chromium, about 5% molybdenum, about 3.5% manganese, about 0.8% beryllium, about 3.0% aluminum, and the balance essentially nickel.

10 11. An alloy suitable in forming partial dentures in accordance with claim 9 which consists essentially of about 15% chromium, about 5% molybdenum, about 3.5% manganese, about 0.8% beryllium, about 3.0% aluminum, about 10% cobalt, and the balance essentially nickel.

15 12. An alloy suitable in forming full dentures in accordance with claim 9 which consists essentially of about 15% chromium, about 5% molybdenum, about 3.5% manganese, about 0.8% beryllium, about 3.0% aluminum, about 20.0% cobalt, and the balance essentially nickel.

20 13. An alloy suitable in forming full dentures in accordance with claim 9 which consists essentially of about 15% chromium, about 5% molybdenum, about 3.5% manganese, about 0.8% beryllium, about 3.0% aluminum, about 5% cobalt and the balance essentially nickel.

25 14. An alloy suitable in forming partial dentures in accordance with claim 9 which contains up to about 3% cobalt.

30 15. An alloy suitable in forming partial dentures in accordance with claim 9 which contains about 12% to 15% cobalt.

#### References Cited

##### UNITED STATES PATENTS

|           |        |               |       |        |
|-----------|--------|---------------|-------|--------|
| 1,942,150 | 1/1934 | Rohn          | ----- | 75—171 |
| 2,072,911 | 3/1937 | Touceda       | ----- | 75—171 |
| 2,089,587 | 8/1937 | Touceda       | ----- | 75—171 |
| 2,206,502 | 7/1940 | Heiligman     | ----- | 75—171 |
| 2,469,718 | 5/1949 | Edlund et al. | ----- | 75—171 |

RICHARD O. DEAN, Primary Examiner

U.S. Cl. X.R.